

E. DOLENSKY.

VACUUM PROCESS FOR PRODUCTION OF STEEL.

APPLICATION FILED OCT. 22, 1912.

1,131,488.

'Patented Mar. 9, 1915.



Witnesses.

Geoffrey MacD. Nairn.

W. Wallace Nairn Jr.

Inventor.

Eugen Dolensky.

By Julian C. Dowell.

his Attorney.

# UNITED STATES PATENT OFFICE.

EUGEN DOLENSKY, OF FRANKFORT-ON-THE-MAIN, GERMANY.

## VACUUM PROCESS FOR PRODUCTION OF STEEL.

1,131,488.

Specification of Letters Patent.

Patented Mar. 9, 1915.

Application filed October 22, 1912. Serial No. 727,122.

*To all whom it may concern:*

Be it known that I, EUGEN DOLENSKY, a citizen of the German Empire, residing at Frankfort-on-the-Main, in the Province of 5 Hesse-Nassau, Prussia, Germany, have invented certain new and useful Improvements in Vacuum Processes for Production of Steel; and I do hereby declare the following to be a full, clear, and exact description 10 of the invention, such as will enable others skilled in the art to which it appertains to make and use the same.

This invention relates to the manufacture of steel of high quality and more particularly to a process for clearing the same.

It is a well known fact that molten steel is much improved if the gases and particles of slag in it are separated and removed, and it is of great importance during this separating and removing, or clearing process that the fluid steel retain its fluidity as long as possible, and in order to bring about this desired result some method for retarding the cooling of the steel must be used.

25 The objects of this invention are two-fold, first to further accelerate the clearing of the steel and second to protect it from rapid cooling, so that it will retain for a long time its fluid state.

30 The accompanying drawing illustrates the form of apparatus which is most generally used in carrying out my process, though I do not wish it to be understood that the invention is limited to the specific details 35 of construction shown therein.

In carrying out my process, the fluid steel is placed in a clearing container A, of the usual size and shape, preferably of iron and lined with a refractory heat insulating material, such as chamotte, and loosely covered 40 with a preferably chamotte cover B. These clearing vessels are then placed in a second container or pit C likewise preferably lined with a refractory material, having a flange c upon the upper edge adapted to have a cover D fastened thereto in an airtight manner, such as by packing. The pit is then exhausted by means of any suitable vacuum pump E and the fluid steel allowed to remain in the pit until the clearing has been 45 completed, after which the pure steel may be poured off. The clearing vessel may if

it is desired have an air pipe or pipes F located therein to equalize the air pressure within the container. It is highly desirable 55 that both the container and pit be heated before the fluid comes in contact therewith, to about the melting point of the steel, and for this purpose I preferably use a flame of water gas, such as is generally used in a 60 Martin furnace for melting the steel, water gas being free from all ashes and sulfur.

The advantages of my invention are manifold; by placing the clearing container in a vacuum, loss of heat is greatly reduced as it 65 is well known that a vacuum gives the best possible protection against loss of heat, and the clearing is greatly accelerated; thus the vacuum serves the double purpose of retaining the heat and accelerating the clearing 70 of the liquid. Besides assisting in the clearing, there is no danger of the steel becoming viscous, even though the container remain in the pit for hours, due to the slow cooling of the liquid. Further the use of the 75 vacuum-pit renders the steel less liable to disturbance during the clearing period, and renders to the greatest possible degree, the certainty of obtaining a perfect quality of steel.

Having thus described my invention what I claim as new and desire to secure by Letters Patent of the United States is:

1. A process for purifying metals, consisting in heating a clearing vessel to the temperature approximately of the molten metal to be purified, placing the molten metal therein and subjecting same to the action of a vacuum, substantially as and for the purpose described.

2. A process for purifying metals, consisting in placing a clearing vessel, heated approximately to the temperature of the molten metal to be purified and containing the molten metal, within a second container, and exhausting said second container, whereby the molten metal is cleared.

In testimony whereof I affix my signature in the presence of two witnesses.

EUGEN DOLENSKY.

Witnesses:

FRIEDRICH CARL WENTZEL,  
MAX HERMANN HÖPPNER.